

# UNITED STATES PATENT OFFICE.

LEWIS E. SAUNDERS, OF NIAGARA FALLS, NEW YORK, ASSIGNOR TO NORTON COMPANY, OF WORCESTER, MASSACHUSETTS, A CORPORATION OF MASSACHUSETTS.

## PURIFYING ALUMINOUS MATERIALS.

1,269,224.

Specification of Letters Patent. Patented June 11, 1918.

No Drawing.

Application filed August 18, 1917. Serial No. 186,922.

To all whom it may concern:

Be it known that I, LEWIS E. SAUNDERS, a citizen of the United States, residing at Niagara Falls, in the county of Niagara 5 and State of New York, have invented certain new and useful Improvements in Purifying Aluminous Materials, of which the following is a specification.

The object of this invention is to provide 10 a method whereby crystalline alumina of relatively high purity may be prepared in the electric furnace from such impure raw materials as calcined bauxite and the like.

It is known that a partial reduction of 15 the non-aluminous oxids normally present in bauxite may be brought about by incorporating with the charge to be fused a small proportion of carbon. If, however, the proportion of carbon be increased to about the 20 amount theoretically necessary for the reduction of all of the oxids of iron, silicon and titanium, it is found that a partial and highly objectionable reduction of alumina occurs. It is customary therefore to use 25 carbon in decidedly less proportion than would be required for a complete reduction of the oxid impurities, with the result that the purification attained is highly incomplete.

30 In a prior Patent No. 960,712, patented June 7, 1910, I have pointed out that this difficulty may be avoided by performing the operation in two stages, in the first of 35 which a substantially complete reduction of the impurities, together with a partial reduction of alumina, is accomplished, while in the second operating stage, performed after the removal of the reduced impurities, the reduction products of alumina 40 are re-oxidized to alumina,—for example, by means of air or other oxidizing gas. In a copending application, Serial No. 186,921, filed Aug. 18, 1917, I have further pointed out that this re-oxidation may be ad- 45 vantageously performed by means of certain solid oxidizing agents, including bauxite.

According to the present invention, a somewhat similar result is accomplished in a single stage by introducing into the charge 50 a relatively large proportion, usually ten to twenty per cent. by weight, or even more, of metallic iron. I have discovered that in presence of metallic iron in sufficient proportions, it is possible to add to the calcined 55 bauxite proportions of carbon up to or

even somewhat exceeding those theoretically necessary for the reduction of the total quantity of non-aluminous oxids (assuming CO as the gaseous reaction product) without appreciable or objectionable reduction 60 of alumina. In practice I prefer to use the carbon in about the theoretical proportion required for the reduction of the non-aluminous oxids. The proportion of iron used increases with increasing percentages 65 of impurities in the bauxite or other alumino raw material, and is therefore, broadly speaking, proportionate to the amount of the carbon addition; although the practice of the method permits of considerable varia- 70 tions in this respect.

The manner in which metallic iron serves to protect the alumina from reduction by carbon is not certainly ascertained. It is of course known that molten iron is an ex- 75 cellent solvent for carbon, and it may be assumed that carbon in solution in iron or combined therewith is incapable of reducing alumina under the conditions existing in the furnace. Also, since molten iron is 80 likewise a solvent for silicon and titanium it is probable that its presence serves, by withdrawing the reduced metals from the field of reaction, to disturb the equilibrium represented by such reversible reactions as— 85



Whatever the explanation may be, I have demonstrated that in presence of sufficient iron it is possible to prepare from a given 90 impure aluminous raw material a product running much higher in alumina, say 97 per cent. and upward, than is obtainable under similar conditions without the use of iron. I have found also that the practice of this 95 process in the manufacture of aluminous abrasives yields a product having a charac- teristic fine grain.

The use of metallic iron in this process presents the great economical advantage 100 over a similar use of iron oxid, together with the added proportion of carbon needed for its reduction, that electrical energy is not con- sumed in a reducing operation which may be carried out at less cost in an ordinary 105 metallurgical furnace. Aside from this con- sideration of cost, quite similar results as regards purity and character of product may be obtained by adding to the calcined bauxite to be fused, in addition to the 110

amount of carbon required for reducing the impurities therein, an added amount of iron oxid equivalent say to ten to twenty per cent. by weight of metallic iron, together with the further quantity of carbon necessary for the reduction of this added iron oxid, or the greater portion thereof.

I claim:—

1. The hereindescribed process of purifying aluminous materials and producing crystalline alumina, which consists in fusing the impure aluminous charge with a proportion of carbon approximating that theoretically required for complete reduc-

tion of the non-aluminous oxids, in presence 15 of metallic iron in sufficient proportion to prevent material reduction of alumina.

2. The hereindescribed process of purifying aluminous materials and producing crystalline alumina, which consists in fusing 20 the impure aluminous charge with a proportion of carbon approximating that theoretically required for complete reduction of the non-aluminous oxids, in presence of upward of ten per cent. by weight of 25 metallic iron.

In testimony whereof I affix my signature.

LEWIS E. SAUNDERS.